

## UNITED STATES PATENT OFFICE

2,610,919

## RUST INHIBITING COMPOSITION

Milton P. Kleinholtz, East Chicago, Ind., assignor  
to Sinclair Refining Company, New York, N. Y.,  
a corporation of Maine

No Drawing. Application June 8, 1946,  
Serial No. 675,443

4 Claims. (Cl. 106—14)

1

My invention relates to compositions which in contact with metals prevent or retard the corrosion thereof. The compositions are especially suitable for preventing the rusting of iron and steel surfaces but may be employed to inhibit the corrosion, due to water or moisture, of non-ferrous metals including copper, brass, bronze, zinc, aluminum, magnesium alloys, and bearing metals, such as copper-lead alloys, nickel alloys, sulfur-nickel alloys, etc.

Some of my compositions may be used as lubricating or hydraulic oils, or, depending upon the concentration of active ingredients, may be added to such oils in such amounts as to impart their corrosion-inhibiting properties thereto; while others are particularly valuable for use, in lieu of the usually-employed slushing oils and other protectorants, in the preservation, for example, of idle machinery, storage drums, castings, tools, spare parts, etc.

A composition according to my invention is prepared by compounding with a mineral oil, such as a petroleum oil, or with a mineral wax or jelly, such as paraffin wax or petrolatum, calcium mahogany sulfonate and alpha-hydroxylauric acid or the product resulting upon the partial self-esterification of such acid.

Calcium mahogany sulfonate is produced by the neutralization with lime of sludge-free, sulfuric acid-treated petroleum oil and is thus distinguished from calcium "green acid" sulfonate obtained by reaction of acid sludge with lime. It is my usual practice to employ the calcium mahogany sulfonate in the form of a concentrate in the oil from which it was derived.

As between the unesterified acid and the partially self-esterified acid, I prefer the latter because it affords somewhat better results. The esterification of alpha-hydroxylauric acid proceeds with the formation of lactide-type compounds as illustrated by the following equations in which R=C<sub>10</sub>H<sub>21</sub>:



In preparing the esterified material for use in the practice of my invention, it is advantageous to so control the esterification that the product mixture predominates in the semi-lactide rather than

2

in the lactide. The reaction is easily effected by heating the acid at a temperature of the order of 200—250° F., most suitably in the presence of a solvent, such as toluene, while providing for the removal of the water of reaction.

For best results, I have found that the concentration of the sulphonate in the mineral oil or wax base should at least slightly exceed the concentration of the acid or partially esterified acid. 10 The total concentration of the two components is determined by practical considerations. Thus, I may prepare oil concentrates for shipping purposes, suitable for subsequent dilution with additional quantities of oil, having much higher concentrations of the addends than are necessary for adequate protection of the particular metal surfaces to be protected. The maximum total concentration of these concentrates is determined only by the solubility of the co-acting materials 20 in the particular oil being employed.

I have determined that, in general, excellent protection is obtained with a sulphonate concentration of from 1—2% on the total weight of the composition and an acid or partially esterified acid concentration on the same basis of from 0.5—1%. My compositions as prepared for use, therefore, generally contain the sulphonate and acid or esterified acid in such concentrations.

Treatment of a metal surface with a composition prepared according to my invention may involve a single or intermittently repeated contact of the surface with the composition or the composition may be maintained in a continuous contact with the surface. Where the composition is applied as a protective coating to articles such as tools, castings, and the like, the method of application is determined by the particular circumstances including the equipment available. In some instances, treatment may be by dipping or immersion, while in other instances, it may be considered most advantageous to spray or brush the surface with the composition. When prepared as a material which is solid at ordinary temperatures, the corrosion-inhibiting composition may in some cases be melted before use, while in other cases it may be applied in the manner of a wax.

My invention is further illustrated by the following examples, which show, inter alia, that my additives co-act in a synergistic manner, the total effect being much greater than the sum of the two effects taken independently. In the test referred to in Examples 1—5, two steel panels measuring about 2" x 3" x 1/8" are sand-blasted to give a fresh metal surface. They are then 50 dipped in the material under test for one minute,

drained 4 hours, and placed in a cabinet maintained at 100% humidity at 120° F. At 24 or 48 hour periods, the panels are inspected for rust spots or areas.

The calcium mahogany sulfonate employed in the experiments on which the examples are based was prepared by treatment of a 200 viscosity mid-continent neutral oil with fuming sulfuric acid, followed by separation of the resulting sludge and reaction of the mahogany acids in the acid oil with lime. The resultant oil after steam reduction to 40% bottoms contained about 25% of calcium mahogany sulfonate and tested as follows:

|                   |       |       |
|-------------------|-------|-------|
| Gravity, API      | 20.0  |       |
| Flash point, °F   | 440   | 15    |
| Fire point, °F    | 510   |       |
| Vis. 100 SSU      | 2083  |       |
| Vis. 210 SSU      | 129.8 |       |
| Four point, °F    | +20   |       |
| Color NPA         | Dark  | 20    |
| Acid No.          | 3.2   | basic |
| Calcium, per cent | 1.46  |       |

The alpha-hydroxylauric acid used in the experiments was prepared in the following manner: 2790 grams (10 moles) of crude alpha-bromo-lauric acid and a solution of 1680 grams (30 moles) of potassium hydroxide in 6.7 liters of water were introduced into a 5 gallon Pfaudler kettle. Upon heating to reflux, the organic phase dissolved completely. The solution was reacted at reflux for about 8 hours. It was then acidified with 3 liters of concentrated hydrochloric acid, with prolonged stirring. The aqueous phase was then drawn off at about 170° F. The crude alpha-hydroxylauric acid was given a second acid wash, followed by two water washes at about 190° F., at which temperature the organic acid is molten and more readily handled. The crude, wet, molten acid obtained analyzed 200 acid number, 0.2% bromine and 0.06% sulfate ash. It weighed 2637 grams, and soon solidified.

In the preparation of the partially self-esterified alpha-hydroxylauric acid tested according to the examples, 2570 grams of the crude alpha-hydroxylauric acid was heated in an open flask over an 8 hour period, the course of the reaction being followed by acid numbers run on hourly samples. The acid number at the end of the 8 hour period was 174 as against 215 after 3 hours heating. The product was an orange-brown oil which solidified at room temperature.

The base oil in the case of Examples 1 to 5 was a solvent extracted Mid-Continent SAE 60 aircraft oil of the following characteristics:

|                          |        |  |
|--------------------------|--------|--|
| Gravity, API             | 26.8   |  |
| Flash point, °F          | 550    |  |
| Fire point, °F           | 625    |  |
| Vis. 100 SSU             | 1751.8 |  |
| Vis. 130 SSU             | 680.4  |  |
| Vis. 210 SSU             | 122    |  |
| Pour point, °F           | +5     |  |
| Color NPA                | 6+     |  |
| ASTM ash, per cent       | 0.00   |  |
| Carbon residue, per cent | 0.36   |  |

#### Example 1

A slushing type oil was prepared by mixing 5 parts of the sulfonate concentrate containing 25% of calcium mahogany sulfonate and 95 parts of the base oil. Duplicate steel panels, coated with the blend, had a humidity cabinet life of less than 100 hours. Only a very slight increase in humidity cabinet life resulted when the quantity of the sulfonate concentrate was increased from 5 parts to 7.5 parts.

#### Example 2

0.5 part of partially self-esterified alpha-hydroxylauric acid was blended with 99.5 parts of the base oil. Panels dipped in this blend and placed in the humidity cabinet rusted in 24 hours. Increasing the amount of the additive to 1% increased the humidity cabinet life to 96 hours.

#### Example 3

0.5 part of unesterified alpha-hydroxylauric acid was mixed with 99.5 parts of the base oil heated at 160° F. Although the acid at the stated temperature appeared to dissolve in the oil, it precipitated upon cooling to room temperature.

A subsequently prepared mixture containing 0.5 part of alpha-hydroxylauric acid, 5 parts of the sulfonate concentrate and 94.5 parts of the base oil remained clear on standing and protected steel panels against rusting in the humidity cabinet for about 300 hours.

#### Example 4

One part of alpha-hydroxylauric acid, 5 parts of the sulfonate concentrate and 94 parts of the base oil were mixed and the blend tested by the humidity cabinet procedure. One panel had a cabinet life of 312 hours, the other a life of 408 hours.

#### Example 5

One part of partially self-esterified alpha-hydroxylauric acid, 5 parts of the sulfonate concentrate and 94 parts of the base oil were mixed and tested by the usual procedure. One panel had a life of 528 hours, the other a life of 408 hours. Increasing the quantity of sulfonate concentrate to 7.5 parts and decreasing the amount of base oil commensurately to 91.5 parts did not increase the humidity cabinet life.

#### Example 6

A blend was prepared containing 71 parts of petrolatum, 23 parts of an East Texas neutral extract, 5 parts of the sulfonate concentrate and 1 part of alphahydroxylauric acid. The blend had the following properties:

|                   |       |  |
|-------------------|-------|--|
| Gravity, API      | 19.8  |  |
| Flash point, °F   | 465   |  |
| Vis. 210 SSU      | 75.2  |  |
| Acid No.          | 1.5   |  |
| Melting point, °F | 157.8 |  |
| Calcium, per cent | .073  |  |
| Sulfur, per cent  | .034  |  |

Duplicate steel panels of the same measurements as the panels of the preceding examples, after sand-blasting, were dipped in the blend which had been heated to 180° F., and allowed to drain overnight. They were then suspended at an angle of 45° to the earth's surface on an unshaded southern exposure. No rust had formed after 30 days.

The East Texas neutral extract and the petrolatum employed in the preparation of the blend had the following properties:

|                   | Neutral Extract | Petrolatum |
|-------------------|-----------------|------------|
| Gravity API       | 11.4            | 33.3       |
| Flash Point °F    | 420             | 555        |
| Fire Point °F     | 485             | 630        |
| Vis. 100 SSU      | 599.4           |            |
| Vis. 210 SSU      |                 | 78.8       |
| Acid No.          |                 | 0.0        |
| Saponification No |                 | 0.84       |
| Melting Point °F  |                 | 164.4      |

## Example 7

The test of Example 6 was repeated with the same result using a blend containing 71 parts of the petrolatum, 23 parts of the neutral extract, 5 parts of the sulfonate concentrate and 1 part of partially self-esterified alpha-hydroxylauric acid.

The properties of this blend were as follows:

|                    |       |
|--------------------|-------|
| Gravity, API       | 20.8  |
| Flash point, °F.   | 485   |
| Vis. 210 SSU       | 74.9  |
| Acid No.           | 1.1   |
| Melting point, °F. | 156.8 |
| Calcium, per cent  | .073  |
| Sulfur, per cent   | 0.33  |

## Example 8

The test of Example 6 was repeated with the same result using a blend containing 71 parts of the petrolatum, 20.5 parts of the neutral extract, 7.5 parts of the sulfonate concentrate and 1 part of partially self-esterified alpha-hydroxylauric acid.

The properties of this blend were as follows:

|                    |       |
|--------------------|-------|
| Gravity, API       | 20.5  |
| Flash point, °F.   | 470   |
| Vis. 210 SSU       | 78.1  |
| Acid No.           | 1.0   |
| Melting point, °F. | 157.0 |
| Calcium, per cent  | 0.111 |
| Sulfur, per cent   | 0.33  |

## Example 9

The test of Example 6 was repeated with the same result using a blend containing 71 parts of the petrolatum, 20.5 parts of the neutral extract, 7.5 parts of the sulfonate concentrate and 1 part of unesterified alpha-hydroxylauric acid.

The properties of this blend were as follows:

|                    |       |
|--------------------|-------|
| Gravity, API       | 20.8  |
| Flash point, °F.   | 475   |
| Vis. 210 SSU       | 75.8  |
| Acid No.           | 1.3   |
| Melting point, °F. | 156.0 |
| Calcium, per cent  | 0.112 |
| Sulfur, per cent   | 0.36  |

## Example 10

The compositions of Examples 6-9, inclusive were employed to coat duplicate steel panels which were subsequently placed in a humidity cabinet maintained at 100° F. and 100% relative humidity. The panels showed no rust after 30 days in the cabinet, although some of them were slightly discolored.

A composition according to my invention may, of course, contain materials other than the sulfonate and acid or partially esterified acid. Thus, in the case of the oil base compositions there

may be present in the oil a viscosity index improver, for example, or a dye to improve the color, or an oxidation inhibitor, or a foam suppressor or all of these. Since calcium sulfonate is an effective detergent, it is usually unnecessary to add a detergent as a separate item when compounding a crank case or other oil to specifications demanding the presence of a detergent.

I claim:

1. A composition adapted to inhibit the rusting of iron and steel consisting essentially of a mineral oil as its base and about 1-2% calcium mahogany sulfonate and about 0.5-1% of a material of the group consisting of alpha-hydroxy lauric acid and the product resulting upon partial self-esterification of such acid and which contains in admixture the acid, the semi-lactide esterification product of the acid, and a relatively minor proportion of the lactide esterification product of the acid.

2. A composition adapted to inhibit the rusting of iron and steel consisting essentially of a base substance from the group consisting of mineral oils and waxes and jellies derived therefrom and about 1-2% of calcium mahogany sulfonate and about 0.5-1% of alpha-hydroxy lauric acid.

3. A composition adapted to inhibit the rusting of iron and steel consisting essentially of a base substance from the group consisting of mineral oils and waxes and jellies derived therefrom and about 1-2% of calcium mahogany sulfonate and about 0.5-1% of the product resulting upon partial self-esterification of alpha-hydroxy lauric acid and which contains in admixture the acid, the semi-lactide esterification product of the acid, and a relatively minor proportion of the lactide esterification product of the acid.

4. A composition according to claim 3 where the partial self-esterification product is that which predominates in the compound formed upon condensation of two molecules of alpha-hydroxy lauric acid with the elimination of one molecule of water.

MILTON P. KLEINHOLZ.

## REFERENCES CITED

The following references are of record in the file of this patent:

## UNITED STATES PATENTS

| Number    | Name         | Date          |
|-----------|--------------|---------------|
| 2,182,992 | Lebo         | Dec. 12, 1939 |
| 2,281,676 | Cook         | May 5, 1942   |
| 2,334,158 | Fuchs et al. | Nov. 9, 1943  |
| 2,348,715 | Adams        | May 16, 1944  |
| 2,383,033 | Adams et al. | Aug. 21, 1945 |
| 2,398,193 | Sharp        | Apr. 9, 1946  |
| 2,403,928 | Kleinholz    | July 16, 1946 |